

3,268,308

## ELECTRODEPOSITION OF A CORROSION RESISTANT DECORATIVE NICKEL-CHROMIUM COATING AND PRODUCTS THEREOF

Thaddeus W. Tomaszewski, Dearborn, and Henry Brown, Huntington Woods, Mich., assignors, by mesne assignments, to The Udylife Corporation, Warren, Mich., a corporation of Delaware

No Drawing. Filed Mar. 1, 1963, Ser. No. 262,199  
17 Claims. (Cl. 29—194)

This invention is for improvements in or relating to decorative nickel electroplating, and more particularly relates to (1) the electrodeposition of sub-microscopic satin-textured to macroscopic satin-textured fine-grained nickel plate from semi-bright and bright nickel plating baths containing dispersed therein fine bath-insoluble particles, and (2) to the exceptional corrosion resistance of these deposits when over-laid with a thin chromium plate.

The decorative fine-grained nickel deposits of this invention have various degrees of brightness, or of uniform smokiness, or of uniform satin-sheen depending mainly on the concentration and particle size of the dispersed fine powders in the semi-bright or bright nickel electroplating baths, the concentration of the nickel brighteners, the degree of agitation of the cathode or the solution, the brightness and smoothness of the metal surface plated upon, and the thickness of the plate applied, and these decorative nickel plates of various degrees of sub-microscopic, microscopic, and macroscopic satin texture and luster when over-laid with a final thin chromium plate provide exceptionally outstanding corrosion protection to the underlying metal.

We have found that the addition to semi-bright and bright nickel electroplating baths of bath-insoluble fine particles of water-insoluble inorganic oxygen-containing titanium and zirconium compounds containing a total of at least three different elements in these compounds and consisting of powders of average particle size less than 5 microns and down to colloidal dimensions will produce exceptionally highly corrosion resistant plate when given the usual final over-lay plate of about 0.01 mil (0.25 micron) of chromium plate. These titanium and zirconium compounds comprise the class consisting of water-insoluble titanates and zirconates of the metals including calcium, strontium, barium, magnesium, nickel, cobalt, iron, zinc, lead, cadmium, cerium, aluminum, antimony and bismuth, the zirconium and titanium silicates, mixtures and mixed compounds thereof, including, for example, the mixed compounds of the zirconates and titanates, the mixed zirconium and titanium silicates, such as the alkali metal titanium or zirconium silicates, the barium, strontium and calcium titanium and zirconium silicates, as for example, barium zirconium silicate and the mixed aluminates, titanates and zirconates, as for example, zirconium spinel, etc. Even concentrations of the fine powders of only about 0.01 gram/liter will make possible improved corrosion protection when the decorative plates obtained from these baths are given a final chromium plate of less than about 0.2 mil (5 microns). With most of these powders the maximum improvement in corrosion protection in the less accessible recessed areas of articles is attained when about 10 to 50 grams/liter of the fine powders are dispersed in the nickel baths, and further increase in concentrations of powder until the baths become quite thick does not improve the already exceptional corrosion resistance when a final thin chromium plate is applied. With the higher concentrations of powder the plates become more satiny up to a point where further increase in concentration of powder produces no further change in appearance of the nickel plate at a given nickel plate thickness on a given base and with a given brightener concentration in the nickel bath. In some cases, as high as

about 500 grams per liter of fine powder can be dispersed in the bath, though in general about 250 grams/liter is the highest that is ever needed for the most macroscopic satin plates.

5 The macroscopic satin-textured types of nickel plate which can be obtained by using the higher concentrations, e.g. about 100 grams/liter or higher of the afore-mentioned powders in the semi-bright and bright nickel electroplating baths are fine-grained lustrous satin nickel deposits which not only have a very pleasing appearance, but which can also be high-lighted by buffing raised areas to give beautiful two-tone effects, and which when chromium plated with about 0.01 mil chromium plate will also provide exceptionally good corrosion protection to the 15 basis metals such as ferrous, aluminum, magnesium, brass, copper, zinc and other metal articles.

The average particle diameter (herein sometimes referred to as "particle size") of the finely powdered bath-insoluble materials should not be greater than 5 microns. 20 As some roughness, especially on shelf areas where particles can settle, may result from the use of materials of particle size greater than about 5 microns, the use of material of particle sizes less than 5 microns are preferred and are advantageous, with the most preferred particle size averaging about 0.02 to about 3 microns as determined with the electron microscope. Some agglomerated particles may have larger particle size than 5 microns but with agitation in the nickel bath the larger agglomerates may be reduced to 5 microns and under. Agitation is usually necessary to keep the fine powder suspended in the baths during plating. Air agitation or mechanical agitation including ultra-sonic agitation of the baths can be used.

Analysis of a satin nickel plate from an air agitated 35 bright nickel bath containing superfine powdered material of particle size of about 0.02 to 3 microns in concentrations even of about 100-200 grams/liter shows usually not higher than about 2.5% of the powdered material uniformly distributed in the nickel plate, and with low concentrations of 10-20 grams/liter or lower of the finest powders, as low as about 0.01% by weight is present in the nickel plate. Microscopic examination of the surface of the plate shows an extremely uniform finely pitted surface which consists of micro-inclusions and micro-pits. 40 Calculations and microscopic examinations indicate that the number of micro-inclusions and micro-pits per square centimeter of surface is at least of the order of  $10^6$ . This textured plate has excellent adhesion, for example, to nickel, ferrous, copper, and brass surfaces similar to that obtained when the nickel bath contains none of the powdered material. The leveling of the bright nickel plate is not decreased by the presence of the finely powdered additives. The throwing and covering power of the agitated bright nickel baths with the suspended powders is about 55 the same as without the fine powders present. It has been found that in plating articles with recessed areas and with shelf areas using particles of the preferred particle size, no objectionable roughness is obtained on the areas on which settling can occur, though in some cases with the larger 60 particle sizes, the shelf areas may be somewhat duller than the rest of the article, though this is usually negligible with short plating times such as 30 seconds to about 5 minutes. With the macroscopic satin nickel the dulling is, of course, no problem.

65 The fine bath-insoluble powders plate out as uniform dispersions in the semi-bright and bright nickel plate and thereby cause sub-microscopic (with the finest particles of 0.01 to about 0.05 micron size) to microscopic-inclusions and sub-microscopic to microscopic-pitting in the 70 surface of the nickel plate. That is at any given instant the surface of the semi-bright or bright nickel plate has distributed over its surface multitudinous fine particles in

various stages of being imbedded in the surface and causing sub-microscopic and microscopic pitting, and with the thinnest plates (flashes or strikes) the pitting is mostly sub-microscopic becoming more microscopically visible with thicker plating. When the usual chromium plate of about 0.01 mil (0.25 micron) chromium is applied to these sub-microscopic to macroscopic satin textured surfaces a very fine favorable porosity pattern is developed in the chromium plate which is the key to the extraordinary corrosion protection afforded to the underlying metal by this composite nickel-chromium plate. With the very fine porosity pattern that is developed in the thin chromium plate there is obtained the very favorable condition of tiny cathode areas, the chromium surrounding the multitudinous tiny anodes (the sub-microscopic and microscopic pits) which results in very weak corrosion currents with very low anodic current densities in the corrosive environments. Thus, the penetration of the corrosion pits towards the underlying basis metal is very greatly diminished. There is also some evidence of extremely fine stress-cracking of the chromium around the micro-inclusions which is also favorable to forming micro cathodes and anodes. There is also the possibility that with the thin chromium plate where most of the micro-inclusions and micro-pits are not completely plated over, that the chromium in the micro-pits may have some chromium chromate inhibitor formed in the micro-pits which would, besides the poorly conducting particles, also be favorable to minimize the start of anodic attack. However, from the results obtained under prolonged severe corrosion exposure it is clear that it is the tiny cathode areas (chromium) surrounding the multitudinous tiny anode (nickel) areas that are the key to the astounding corrosion protection afforded by the thin chromium plated sub-microscopic-to-macroscopic-textured fine-grained nickel deposits of this invention.

These textured nickel deposits give the best appearance and corrosion protection results when plated on top of semi-bright sulfur-free nickel or bright nickel deposits. It is best and also simpler to use the regular semi-bright nickel plating baths for most of the plate and to use the minimum of the textured nickel plate required to obtain the desired appearance and corrosion resistance, because the textured nickel plating bath requires added control due to the presence of the dispersed particles, and also because the best corrosion protection results are obtained in this way.

The mechanism by which the particles plate out is not clear, the adsorption of hydrogen ions and nickel ions by the particles would give the particles a positive charge and in this way they would tend to plate out. Also, under the powerful reducing conditions at the nickel cathode, it might be possible that the particles which are not semiconductors could become semi-conductors by partial reduction. Nevertheless, independent of the mechanism of the plating out of these particles into the nickel plate, it is amazing how readily these particles plate out in a surprisingly uniform manner in semi-bright and bright nickel plates. The plating out of the fine particles starts immediately and in the bright nickel plating baths there is evidence that the first layers of nickel plated out actually contain somewhat higher concentrations of the fine powder than the subsequent ones. Also, the first layers may cause more micro-stress cracking in the thin chromium than the subsequent layers.

The macroscopic satin nickel plate obtained from the agitated bright or semi-bright nickel plating baths containing the higher concentrations of these fine powders can as already mentioned be easily buffed to a high luster, without losing the exceptional corrosion resistance when chromium plated. Thus, the beautiful two-tone effects achieved by buffing accessible portions of the macroscopic satin nickel plated object still have the highest corrosion resistance after the final chromium plate. Another useful decorative effect can be obtained where brush or

polishing lines are desired in a satin finish, by using coarse polishing grit, for example, 120 to 150 emery on the basis metal. The original coarse polishing lines, although diminished by the high leveling satin nickel plate, are still visible. In this way, a highly corrosion resistant scratch brush finish satin nickel is obtained without having to resort to scratch brushing a final nickel plate and thus greatly decreasing its corrosion protection.

Before technical grade powders are used commercially they should always be checked first in small scale tests such as in 1-4 liter baths before being added to large baths because certain harmful impurities such as metallic powders or too coarse particles may be present which will cause rough plate, especially on shelf areas, but otherwise technical grade fine powders normally produce results similar to those obtained from the use of high purity grades of the same particle size and structure. Also, if the powder is not wetted properly by the nickel bath, it should be washed with solvents and checked for freedom from fatty or oily films.

In general, bright or semi-bright nickel plating baths of the Watts, sulfate, high chloride, sulfamate or fluoroborate type, or mixtures can be used. While boric acid is the buffer usually used, other buffers, such as formates, acetates, succinates or citrates may also be employed.

The pH of the baths may be from about 2 to 6, though the preferred pH values are from about 3.5 to 5.2. The temperature of the baths can be from room temperature to at least 80° C., though in general a temperature of about 55° C. to about 65° C. is preferred.

The best addition agents or brighteners to achieve the semi-bright and bright nickel plating conditions necessary to obtain the lustrous satin textured nickel after the addition to the bath of the afore-mentioned powders are the following: the sulfur-containing brighteners including aromatic and unsaturated aliphatic sulfonic acids, sulfonamides and sulfonimides, such as the benzene- or naphthalene-sulfonic acids, p-toluene sulfonimide, benzene sulfonamide, o-benzoyl sulfimide, vinyl sulfonic acid, allyl sulfonic acid, 2-butyne-1, 4-disulfonic acid, o-sulfobenzaldehyde, etc.; the addition agents which produce semi-bright sulfur-free nickel plate such as formaldehyde, chloral hydrate, bromal hydrate, coumarin, butyne diol, adducts of butyne diol, used alone or in combination; combinations of unsaturated addition agents containing unsaturated linkages such as



$\text{C}=\text{C}$ ,  $\text{C}=\text{N}$ ,  $\text{C}\equiv\text{C}$ ,  $\text{C}\equiv\text{N}$ , with organic sulfur-containing brighteners, organic sulfon-compounds, and combinations of the latter with small concentrations of amines, such as quinaldine, polyamines or unsaturated amines such as N-allyl isoquinolinium bromide, or other quaternaries of pyridines or quinolines or isoquinolines.

Cobalt and iron can be present in the nickel bath as cobalt or ferrous sulfates, chlorides, bromides, sulfamates or fluoroborates in concentrations as high as at least 40 grams/liter, yielding nickel alloy plates containing concentrations of cobalt and/or iron up to a total of about 50% and it is to be understood that, except when the context requires otherwise, the expression "nickel plate" as used herein covers such nickel alloy plates.

Surface active agents may be present in the baths, but are not usually necessary in the air agitated baths.

The maximum increase in lustrous sheen is obtained when the fine powders are used in the agitated full bright nickel plating bath such as the air-agitated bright nickel plating baths possessing good leveling properties. Less luster is obtained when the nickel baths contain only a carrier type brightener such as a benzene or naphthalene sulfonic acid, p-toluene sulfonamide, benzene sulfonamide or o-benzoyl sulfimide. In the latter cases the luster is flatter. This is also true when the semi-bright sulfur-free type of addition agent such as formaldehyde coumarin,

chloral hydrate or bromal, is used solely with the fine powders, and with these semi-bright addition agents it is usually best to use the ultra-fine particle size powders of less than 0.5 micron particle size, and preferably less than 0.5 micron particle size as determined with the electron microscope.

The sub-microscopic to macroscopic satin-textured nickel plate accepts chromium plate like regular nickel plate, and in general only the usual thicknesses of final chromium layer need be used, that is 0.25 micron though thicknesses of 2.5 or 5 microns may be used. Besides, the decorative nickel finish as such, or with the usual final chromium finish, the microscopic to macroscopic satin-textured nickel plate can be given a rhodium, silver, tin, brass, bronze, copper, gold, or tin-nickel (65-35) alloy or other final thin coating. Thin wax, resin, or "soluble wax," films or clear lacquers greatly decrease finger marking of the final coatings, such as nickel, bronze, silver or brass coatings. Chromium, rhodium, and tin-nickel alloy plate do not need these organic coatings, at least not for tarnishing effects.

Below are listed examples of baths of this invention in which one or more of the above described powdered materials may be used as described herein. It is to be understood that other inorganic bath compositions and other brighteners may be used, though one of the preferred class of brighteners is the organic sulfon compounds.

#### Example I

|                                                                                                         | Grams/liter |
|---------------------------------------------------------------------------------------------------------|-------------|
| Strontium titanate and/or zirconate<br>(SrTiO <sub>3</sub> , SrZrO <sub>3</sub> ), 0.05 to 3 micron av. |             |
| particle size                                                                                           | 0.1-100     |
| NiSO <sub>4</sub> ·6H <sub>2</sub> O                                                                    | 200-300     |
| NiCl <sub>2</sub> ·6H <sub>2</sub> O                                                                    | 40-120      |
| H <sub>3</sub> BO <sub>3</sub>                                                                          | 40          |
| o-Benzoyl sulfimide                                                                                     | 1-4         |
| p-Toluene sulfonamide                                                                                   | 1-2         |
| Allyl sulfonic acid                                                                                     | 1-4         |
| 2-butynoxy-1, 4-diethane sulfonic acid                                                                  | 0.05-0.2    |
| pH=3.5-5.2, temp. 50°-70° C.                                                                            |             |
| Air agitation.                                                                                          |             |

#### Example II

|                                                                       |            |    |
|-----------------------------------------------------------------------|------------|----|
| Barium titanate and/or zirconate<br>0.1 to 3 micron av. particle size | 0.2-100    | 50 |
| NiSO <sub>4</sub> ·6H <sub>2</sub> O                                  | 200-300    |    |
| NiCl <sub>2</sub> ·6H <sub>2</sub> O                                  | 40-80      |    |
| H <sub>3</sub> BO <sub>3</sub>                                        | 40         |    |
| Benzene sulfonamide                                                   | 1-3        | 55 |
| Allyl sulfonic acid                                                   | 1-4        |    |
| N-allyl quinaldinium bromide                                          | 0.003-0.01 |    |
| pH=3.5-5.2, temp. 50°-70° C.                                          |            |    |
| Air agitation or mechanical agitation.                                |            | 60 |

#### Example III

|                                                                             |          |    |
|-----------------------------------------------------------------------------|----------|----|
| Zirconium silicate (ZrSiO <sub>4</sub> )<br>av. particle size 0.1-5 microns | 5-200    | 65 |
| NiSO <sub>4</sub> ·6H <sub>2</sub> O                                        | 200-300  |    |
| NiCl <sub>2</sub> ·6H <sub>2</sub> O                                        | 40-100   |    |
| H <sub>3</sub> BO <sub>3</sub>                                              | 40       |    |
| Benzene sulfonamide                                                         | 1-3      |    |
| o-Benzoyl sulfimide                                                         | 1-4      | 70 |
| Allyl sulfonic acid                                                         | 1-3      |    |
| 2-butynoxy-1, 4-diethane sulfonic acid                                      | 0.05-0.2 |    |
| pH=3.0-5.2, temp. 50°-70° C.                                                |          |    |
| Air agitation.                                                              |          | 75 |

#### Example IV

|                                                                        |            |
|------------------------------------------------------------------------|------------|
| Cerium titanate and/or zirconate<br>av. particle size 0.1 to 3 microns | 0.2-150    |
| 5 NiSO <sub>4</sub> ·6H <sub>2</sub> O                                 | 50-150     |
| NiCl <sub>2</sub> ·6H <sub>2</sub> O                                   | 200-100    |
| H <sub>3</sub> BO <sub>3</sub>                                         | 40         |
| o-Benzoyl sulfimide                                                    | 2-4        |
| 10 N-allyl isoquinolinium bromide                                      | 0.003-0.01 |
| pH=3.5-5.2, temp. 50°-70° C.                                           |            |
| Air agitation.                                                         |            |

#### Example V

|                                                                            |           |
|----------------------------------------------------------------------------|-----------|
| 15 Strontium titanate and/or zirconate<br>av. particle size 0.05-3 microns | 0.2-100   |
| NiSO <sub>4</sub> ·6H <sub>2</sub> O                                       | 200-300   |
| NiCl <sub>2</sub> ·6H <sub>2</sub> O                                       | 30-60     |
| 20 H <sub>3</sub> BO <sub>3</sub>                                          | 40        |
| Bromal and/or chloral hydrate                                              | 0.05-0.1  |
| Formaldehyde                                                               | 0.02-0.08 |
| pH=3.5-5.2, temp. 50°-65° C.                                               |           |
| Air agitation or mechanical agitation.                                     |           |

#### Example VI

|                                                                            |          |
|----------------------------------------------------------------------------|----------|
| Strontium titanate and/or zirconate<br>av. particle size of 0.05-3 microns | 0.2-10   |
| 30 Ultra-fine silica powder (Quso)                                         | 1-50     |
| NiSO <sub>4</sub> ·6H <sub>2</sub> O                                       | 200-300  |
| NiCl <sub>2</sub> ·6H <sub>2</sub> O                                       | 30-100   |
| H <sub>3</sub> BO <sub>3</sub>                                             | 40       |
| o-Benzoyl sulfimide                                                        | 0.1-3    |
| Benzene sulfonamide                                                        | 1-3      |
| Allyl sulfonic acid                                                        | 1-4      |
| 2-butynoxy-1, 4-diethane sulfonic acid                                     | 0.05-0.2 |
| pH=3.5-5.2, temp. 50°-70° C.                                               |          |
| Air agitation or mechanical agitation.                                     |          |

When the ultra-fine particles of about 0.01 to 0.05 micron size particles are used in the semi-bright and bright nickel electroplating bath, it is difficult to see the included particles in cross-section of the nickel plate even at the highest magnification of the light microscope. However, on the surface of the plate using strong light it is possible to just see the microscopic pitting effect of these sub-microscopic particles. The thinner the plate that is deposited on a bright surface, the more difficult is it to distinguish any difference between the appearance of the textured deposit and the bright plate obtained without the particles present. With increasing thickness of the deposit and with increasing concentrations of the fine particles, the micro-inclusions and micro-pitting can be more easily discerned, and an increasing degree of visible satin texture of the plate occurs. Thus, in the above examples of baths of this invention, the lower concentrations of powder of 0.2 to about 20 grams/liter, and in some cases even to about 50 grams/liter are best for obtaining bright plate from the bright nickel baths, and can thus be used best for very thin plates of about 0.01 to 0.1 mil thickness on top of regular bright nickel or semi-bright nickel plate to obtain after the final chromium plate very high corrosion protecting bright plate. Using the CASS and Corrodkote accelerated corrosion tests, many cycles are passed with only 0.6 mil of regular bright nickel or semi-bright nickel that is given a thin plate (0.01 to 0.1 mil) from the baths illustrated in the above examples, and a final 0.01 mil chromium plate; whereas, with regular bright nickel alone of the same total plate thickness and the same final thin chromium plate, not one cycle is passed. With the higher concentrations of powder and with thicker deposits (0.2 mil to 0.5 mil) the

plate becomes more macroscopically satin-textured, and the extremely excellent corrosion protection is maintained when the same thin final chromium plate is applied. Again, the best corrosion protection results are obtained when the textured plate of this invention is applied on top of regular nickel plate which can be dull, semi-bright or bright nickel plate depending on the decorative effect desired. That is, the degree of brightness, smokiness, or satin quality is dependent on the original brightness and smoothness of the surface plated upon, as well as the thickness of the plate applied, the concentration and type of brighteners present, the concentration of the powder in the bath, the particle size of the powder and the type of powder, that is, its chemical constitution. As an illustration of the latter, barium titanate at a given concentration, for example, of 20 grams/liter and with an average particle size of, for example, 0.5 to 3 microns, will give a more macroscopic satin nickel plate than will strontium titanate at the same concentration and of the same average particle size and from the same bright nickel bath. By increasing the concentration of the strontium titanate or by using lower concentrations of the brighteners, then the degree of macroscopic satin texture will be more closely alike. Furthermore, magnesium titanate of the same average particle size will require even higher concentrations of the powder to produce the same degree of macroscopic satin texture as the strontium titanate, or conversely strontium titanate and even more so magnesium titanate will allow a full bright plate from the bright nickel bath at higher concentrations of powder than will barium titanate.

The nickel brighteners that produce very high leveling and brilliance as, for example, those given in U.S. 2,647,866 (Aug. 4, 1953) and U.S. 2,800,440 and 2,800,443 (July 23, 1957) will produce the highest brilliance with the powders dispersed in these bright nickel baths. For less luster, either the higher concentrations of the powders can be used in the very bright plating baths or lower concentrations or with just the organic sulfon-compounds present as brighteners. These latter brighteners such as o-benzoyl sulfimide, o- or p-toluene sulfonamide, naphthalene, mono-, di-, or tri-sulfonic acids, etc., can be used in concentrations ranging from about 0.1 gram/liter to saturation.

In the case of barium, strontium and calcium titanates and zirconates, in the sulfate containing nickel baths such as the Watts nickel bath, there is also formed to a certain extent the insoluble sulfates of these alkaline earth metals from the slight solubility of the titanates and zirconates in the acidic bath. However, this causes no problems in appearance effects or corrosion resistance results, and in the case of strontium zirconate and titanate it seems to be a beneficial effect in that the mixed strontium sulfate, strontium titanate or strontium zirconate fine particles give extremely excellent corrosion protection results even in very deeply recessed areas where the plate is very thin and is just barely covered with the final chromium plate. Many mixtures of fine powders as well as mixed fused powders give very good results, especially for the best distribution of micro-inclusions and micro-pits in recessed areas. For example, strontium zirconate with zirconium silicate; aluminum oxide with zirconium silicate; ferric oxide or ferrates or aluminates with titanates or zirconates. With ultra-fine silica which is the best powder for sub-microscopic pitting and the least dulling effects excellent results can be obtained. For example, with strontium titanate it is best to use about 5 to 50 grams per liter of very fine silica to about 0.05 to 1 gram per liter of 0.1 to 3 micron strontium titanate to obtain sub-microscopic to microscopic textured fully bright nickel plate from the bright nickel bath and for macroscopic textured semi-bright nickel to use 1 to 10 grams per liter of the very fine silica powder to about 10 to 50 grams per liter of the strontium titanate, or zirconate.

To achieve the highest possible corrosion protection

results with the textured decorative nickel plate of this invention on complex shaped articles such as many zinc die-cast articles, for example, rear view mirror holders, intricate light housings, steel bumpers, hub caps, and grilles, it is best to use duplex or dual nickel underneath the textured nickel deposit. Thus, the total nickel deposit would consist of semi-bright sulfur-free nickel followed by regular bright nickel followed by a thin textured nickel deposit of this invention. The latter being used as thin plate (0.01 to about 0.1 mil) if the highest brilliance is desired, or as a thicker plate with more powder in the bath to obtain a more subdued brightness or satin type of finish if desired. When ductile copper plate is used under nickel plate that has a final coating of the textured decorative nickel plate of this invention, then the copper plate also helps in the total corrosion resistance unlike the case when copper is used as a substitute for part of the bright nickel thickness in deposits of copper-bright nickel and the usual 0.01 mil thick final chromium. It is believed that this beneficial effect of copper is also due to the tiny cathode areas developed in the final thin chromium plate, which in turn is due to the fine favorable porosity pattern developed in the thin final chromium plate as a result of its being deposited over a decorative nickel surface containing multitudinous sub-micro to micro-inclusions and sub-micro to micro-pits of the order of  $10^6$  per sq. cm.

A particularly desirable and extremely corrosion resistant composite plate is formed by electroplating the nickel plate of this invention on the upper layer of the composite nickel coating described and claimed in co-pending application Serial No. 103,296, filed April 17, 1961, which is assigned to the assignee of this invention now U.S. Patent 3,090,733, issued May 21, 1963. This composite plate comprises a lower nickel plate having an average thickness of about 0.15 mil to about 1.5 mils and an average sulfur content less than about 0.03%, a first overlying electroplate of nickel, or nickel-cobalt alloy containing at least about 50% nickel and having a thickness of about 0.005 mil to about 0.2 mil and an average sulfur content of about 0.05% to about 0.3%, a second overlying layer of nickel or nickel-cobalt alloy containing at least about 50% nickel having a thickness of about 0.15 mil to about 1.5 mils and an average sulfur content of about 0.02% to about 0.15%, the second overlying layer containing a lower percentage of sulfur than said first overlying nickel electroplate and a higher percentage of sulfur than said lower nickel plate, an overlying layer of the nickel plate of this invention, and a top or upper layer of chromium having a thickness less than about 5 microns. In this composite plate, the fine grain nickel plate of this invention may vary from a thin flash layer to the thicker plate characterized as the macroscopic satin textured plate, but even the thin flash plates of this invention in such composite plate give excellent corrosion resistance.

Certain of the titanates tend to raise the pH of the nickel baths to pH values around 5.5, as for example, magnesium titanate, iron titanates, and it is therefore best to use these higher pH values with such powders. The copper, zinc, cadmium, lead, antimony and bismuth titanates and zirconates must be used with much more careful control than the other powders to avoid an excess of free copper, zinc, lead, etc., ions which are known to be harmful to the quality of the nickel deposit, and thus it is best to use these powders at the lowest concentrations (0.1 to 1 gram/liter) for the microscopic satin-textured lustrous nickel plate, and to use the higher pH values of the nickel bath to minimize solubilization. In general, the preferred powders are the calcium, strontium, barium, magnesium, nickel, cobalt, iron, cerium and aluminum zirconates and titanates, zirconium silicate, and the calcium, strontium, magnesium, and barium zirconium silicates, and the best of these are the strontium and barium zirconates and titanates, zirconium silicate, and the strontium and barium zirconium silicates. These powders are

by far the least critical to use from the standpoint of their concentrations in the baths, the pH values of the baths, e.g. 3-6, and give optimum results for both microscopic and macroscopic satin-textured lustrous nickel plate.

What is claimed is:

1. A method for electrodepositing a decorative nickel plate which comprises the step of electrolyzing an aqueous acidic solution of at least one nickel salt selected from the group consisting of nickel sulfate, nickel chloride, nickel fluoborate and nickel sulfamate and at least one soluble organic addition agent capable of producing semi-bright to fully bright nickel plate, said solution containing dispersed therein about 0.1 to about 250 grams/liter of at least one material selected from the class consisting of the water-insoluble oxygen-containing titanium and zirconium compounds containing a total of at least three different elements, said material being in the form of a fine powder having an ultimate particle size less than about 5 microns average diameter, thereafter plating on said electrodeposited layer an overlayer of a metal selected from the group consisting of chromium, rhodium, silver, tin, brass, bronze, copper, gold, and an alloy consisting of 65 tin and 35 nickel, said overlayer having a thickness less than about 5 microns.

2. A method for electrodepositing a decorative nickel plate which comprises the step of electrolyzing an aqueous acidic solution of at least one nickel salt selected from the group consisting of nickel sulfate, nickel chloride, nickel fluoborate and nickel sulfamate and at least one soluble organic addition agent capable of producing semi-bright to fully bright nickel plate, said solution containing dispersed therein about 0.1 to about 250 grams/liter of at least one material selected from the group consisting of the water-insoluble titanates and zirconates of a metal selected from the group consisting of calcium, strontium, barium, magnesium, nickel, cobalt, iron, and aluminum, the zirconium and titanium silicates, and mixtures and mixed compounds thereof, said material being in the form of a fine powder having an ultimate particle size of less than about 5 microns average diameter, thereafter plating on said electrodeposited layer an overlayer of a metal selected from the group consisting of chromium, rhodium, silver, tin, brass, bronze, copper, gold, and an alloy consisting of 65 tin and 35 nickel, said overlayer having a thickness less than about 5 microns.

3. A method in accordance with claim 1 wherein said fine powder is strontium titanate.

4. A method in accordance with claim 1 wherein said fine powder is barium titanate.

5. A method in accordance with claim 1 wherein said fine powder is zirconium silicate.

6. A method in accordance with claim 1 wherein said fine powder is strontium zirconate.

7. A method in accordance with claim 1 wherein said fine powder is barium zirconate.

8. A method in accordance with claim 1 wherein said fine powder is barium zirconium silicate.

9. A method in accordance with claim 1 wherein the metal of said overlayer is chromium.

10. A method for electrodepositing a decorative nickel plate which comprises the step of electrolyzing an aqueous acidic solution of at least one nickel salt selected from the group consisting of nickel sulfate, nickel chloride, nickel fluoborate and nickel sulfamate and at least one soluble organic addition agent capable of producing semi-bright to fully bright nickel plate, said solution containing dispersed therein about 0.1 to about 250 grams/liter of a mixture of at least one material selected from the group consisting of the water-insoluble titanates and zirconates of a metal selected from the group consisting of calcium, strontium, barium, magnesium, nickel, cobalt, iron, and aluminum, the zirconium and titanium silicates, mixed compounds thereof and about 1 to about 50 grams/liter of finely divided silica powder, said materials being in the form of fine powders having an ultimate particle size of less than about 5 microns average diameter, and an electrodeposited overlayer of a metal selected from the group consisting of chromium, rhodium, silver, tin, brass, bronze, copper, gold, and an alloy consisting of 65 tin and 35 nickel, said overlayer having a thickness in the range of about 0.25 to about 5 microns.

size of less than about 5 microns average diameter, thereafter plating on said electrodeposited layer an overlayer of a metal selected from the group consisting of chromium, rhodium, silver, tin, brass, bronze, copper, gold, and an alloy consisting of 65 tin and 35 nickel, said overlayer having a thickness less than about 5 microns.

11. A method in accordance with claim 2 wherein said nickel plate is electrodeposited directly on an electrodeposit consisting essentially of nickel.

12. A method in accordance with claim 2 wherein said dissolved organic nickel brightener is selected from the group consisting of aromatic and unsaturated sulfonic acids, sulfonamides and sulfonimides.

13. A method in accordance with claim 2 wherein said dissolved organic nickel brightener is o-benzoyl sulfimide.

14. A composite electroplate on a metal surface susceptible to atmospheric corrosion which comprises a nickel plate with chromium overplate, said nickel plate having been electrodeposited from an acidic nickel plating bath containing dissolved therein at least one organic nickel brightener capable of producing semi-bright to fully bright nickel plate, and having dispersed in said bath at least 0.1 gram/liter of at least one water-insoluble powder material selected from the class consisting of the water-insoluble oxygen-containing titanium and zirconium compounds containing a total of at least three different elements, said powder material having particles of average ultimate particle size less than about 5 microns, and an electrodeposited chromium overlay plate on said nickel plate of less than about 5 microns thickness.

15. A composite electroplate in accordance with claim 14 wherein said nickel plate directly overlies an electrodeposit consisting essentially of nickel.

16. A composite electroplate in accordance with claim 14 wherein said dissolved organic nickel brightener is selected from the group consisting of aromatic and unsaturated aliphatic sulfonic acids, sulfonamides and sulfonimides.

17. A composite electroplate on a metal surface susceptible to atmospheric corrosion which comprises a lower nickel electroplate having a thickness of about 0.15 mil to about 1.5 mils and an average sulfur content less than about 0.03%, an overlying layer consisting essentially of an electroplate selected from the group consisting of nickel electroplate and nickel cobalt alloy electroplate containing at least about 50% nickel and having a thickness of about 0.005 mil to about 0.2 mil and an average sulfur content of about 0.05% to about 0.3%, an overlying layer consisting essentially of an electroplate selected from the group consisting of nickel electroplate and nickel-cobalt alloy electroplate containing at least about 50% nickel, and having a thickness of about 0.15 mil to about 1.5 mils and an average sulfur content of about 0.02% to about 0.15%, the second overlying layer containing a lower percentage of sulfur than the said first overlying nickel electroplate and a higher percentage of sulfur than said nickel plate, an overlying layer of nickel plate electrodeposited thereon from an acidic nickel plating bath containing dissolved therein at least one organic nickel brightener capable of producing semi-bright to fully bright nickel plate and having dispersed therein about 0.1 to about 250 grams/liter of at least one material selected from the class consisting of water-insoluble oxygen-containing titanium and zirconium compounds containing a total of at least three different elements, said material being in the form of a fine powder having an ultimate particle size less than about 5 microns average diameter, and an electrodeposited overlayer of a metal selected from the group consisting of chromium, rhodium, silver, tin, brass, bronze, copper, gold, and an alloy consisting of 65 tin and 35 nickel, said overlayer having a thickness in the range of about 0.25 to about 5 microns.

11

**References Cited by the Examiner**  
**UNITED STATES PATENTS**

2,739,085 3/1956 McBride ----- 204—181 X  
2,771,409 11/1956 Cross ----- 204—40 X  
3,057,048 10/1962 Hirakis ----- 204—49 X  
3,061,525 10/1962 Grazen ----- 204—9

12

3,090,733 5/1963 Brown ----- 204—40  
3,132,928 5/1964 Crooks et al. ----- 204—40 X

JOHN H. MACK, *Primary Examiner.*  
HOWARD S. WILLIAMS, *Examiner.*  
G. KAPLAN, *Assistant Examiner.*